

# UNITED STATES PATENT OFFICE.

HUGH RODMAN, OF EDGEWOOD, PENNSYLVANIA, ASSIGNOR TO RODMAN CHEMICAL COMPANY, A CORPORATION OF PENNSYLVANIA.

## METHOD OF MAKING LOW-DENSITY COKE PRODUCTS.

1,283,310.

Specification of Letters Patent.

Patented Oct. 29, 1918.

No Drawing.

Application filed February 7, 1917. Serial No. 147,099.

To all whom it may concern:

Be it known that I, HUGH RODMAN, a citizen of the United States, and a resident of Edgewood, in the county of Allegheny and 5 State of Pennsylvania, have made a new and useful Invention in Methods of Making Low-Density Coked Products, of which the following is a specification.

This invention relates to the production 10 of low density coked products and discloses a new and improved method of making such products.

Efforts have been made to make low density products by heating a coking material or a mixture containing coking material in such a way as to produce masses of light, porous coked material, these masses being generally crushed and screened to obtain the size of product desired. As this 20 process is particularly applicable to the production of carburizing material, I will describe it in that connection, though the art is also applicable to the production of filtering material, filling for reaction towers, etc.

25 Limiting the description further to the use of a single coking material, I will describe a process which I have used commercially for the production of light, coked, carburizing material and then describe the 30 new and improved process forming the basis of this patent application.

I have hitherto made light, coked carburizing material by mixing a mass of finely powdered coking coal with powdered energizers, such as lime and soda ash, and then feeding this mixture into a heated revolving kiln, so that the mixture was coked while tumbling. In this way I have produced excellent carburizing material, but in general 40 have found great difficulty in regulating the operation so as to avoid the production of dust and oversized material. The object aimed at was the production of light coked masses about one quarter inch in diameter, 45 but there would always be considerable material in lump larger than desired and also considerable small material and dust. The oversized lump could of course be crushed to proper size, but in doing so more dust was 50 produced, and the dust was generally waste or required further, expensive treatment.

My present invention is a process of making such light coked products practically

without waste and in a way that allows of great flexibility both in manufacturing and 55 in the character of product produced. That is, it gives a means of making the material without the production of dust and also makes it possible and easy to produce material of any density desired. It also produces an improved light coked product in that the finished product has a comparatively smooth surface, differing from the edged and angular product obtained by crushing, and therefore less liable to produce 60 dust in handling. It also makes possible the production of a very uniformly sized product, as the material, in this new process, is sized before being coked, and the uncoked oversize and undersize material can 65 be easily manipulated to produce proper sized uncoked material; in this way avoiding 70 all waste.

The new process consists in forming the raw material into pellets or fragments of 75 proper size and so made that they will, when heated quickly, expand in size, or at least not contract, and coke to a firm material of the size desired without breaking up or adhering to neighboring fragments and without 80 producing any considerable dust.

Before describing the process further, I will explain that I have hitherto made carburizing material by fashioning coking material, or a mixture containing coking 85 material, into pellets or fragments and have then coked them, either before or during use as a carburizing agent, to produce small unit masses of coked material. This old process differs from the present one in that the pellets or fragments produced were of such construction and coked in such a way that the resultant coked product generally occupied a much smaller volume after coking than before. In other words, each small 95 fragment or pellet would shrink in volume during the coking process till it occupied roughly, 60% to 75% of its original raw volume; and the final product was therefore, generally dense and heavy.

I now find that by coking the pellets or fragments as originally made, but much more rapidly than was customary, and also by changing the formula of the mixture and then coking rapidly, I can cause each individual pellet or fragment to expand in size 100 to 105

2  
during the coking process, instead of shrinking as heretofore, and at the same time cause it to substantially maintain its original contour. In this way I produce excellent carburizing material of low density and without waste.

As a concrete example I will state that I have heretofore made pellets or fragments by fashioning a mixture of one hundred 10 parts finely powdered coking coal, ten parts of soda ash and fifteen parts of lime, using a molasses solution as binding agent, and generally tumbling the material to produce small pellets or pills about one-fourth inch 15 in diameter. These were sometimes dried by gentle heat and then used direct as a carburizing agent, or they were sometimes fed into the cold end of a rotating kiln and gradually dried and coked and discharged 20 at the hot end. In either case there was a loss in weight of about 35% (due to the vaporizing of the water, loss of gas by the coal and reduction of the lime and soda ash) and also a loss in volume of about 35%. The 25 net result was the production of raw pills with a density of about 70 (figuring water as 100 dense) when measured in bulk, which, in coking, lost 35% in volume and 35% in weight, leaving finally a coked product having 30 65% the original weight and still having a density of 70. (The density is that of a pile of pellets rather than of a single pellet; that is, a pint of the pellets weighed 70% of the weight of a pint of water).

35 In carrying out the new process I first dry the pills (if that be necessary) and then heat them very rapidly, generally agitating them at the same time to destroy any light adhesions. In this way I am able to overcome 40 the excessive shrinkage of the old method, and instead of the pellets losing volume they either hold their original volume or else increase in volume, so that by this new process I can easily make a product with a density of 30 and can vary the density to produce lighter or heavier pellets as desired.

The new process of coking very rapidly can be applied to the pellets as formerly compounded, but I prefer to make the pellets for this new process with a weaker bond 50 than before. When lime and molasses solution are used there is a setting or hardening effect due to the reaction of these two materials, so that in coking the expanding force 55 of the pent in gases has to overcome this strong bond. For this reason I prefer to use powdered marble dust instead of lime with molasses solution and to use a weaker solution of molasses. As an improvement 60 beyond this, I may prefer to use a binding agent having considerable value as a coke producer and I find ordinary tar will serve excellently. I may make the pellets by tumbling the mixture of powdered coal, lime- 65 stone and soda ash (as 100 parts of coal, 10

parts of soda ash and 15 parts of limestone) with liquid tar so as to fashion small pellets or pills; these are screened to secure the sizes desired and then fed into a revolving furnace or kiln maintained at about 1500° 70 F. The volatile matter from the tar and the coal burn above the tumbling mass and maintain, or help to maintain, the proper temperature and the individual pellets are coked quickly, expanding as before described, and finally discharging into a cooling device. The form of the heating devices for coking the pellets rapidly forms no part of this invention, but I find a satisfactory device to consist of a rotating furnace so 80 arranged that the incoming pellets fall directly into a considerable mass of tumbling pellets already coked and hot. I can accomplish the same purpose of coking rapidly by feeding the pellets into an ordinary rotary 85 kiln, taking care to see that they quickly reach a coking zone; that is, the ordinary cold, feed end of the kiln is maintained at or near a coking temperature.

I have described one method of making 90 the pellets or fragments, one mixture, one device for coking, etc., and also one object—the production of light carburizing material, but I conceive of my invention as broader than these limitations. I have also 95 spoken of the pellets increasing in volume or at least not shrinking. It will be apparent that they might be compounded or manipulated so as to shrink slightly and still mark an advance over the excessive shrink- 100 age of the old processes.

I have also spoken of tar and its coking properties, but it will be apparent to those skilled in such matters, that other coking materials, as heavy oil or heavy molasses 105 may be used. Also the total coking material in the raw pellet or fragment may be the binder, as the tar, the rest of the carbonaceous material in the pellet being non-coking, as charcoal dust.

110 What I claim is:

1. The process of making low density products which consists in fashioning coking material or a mixture containing coking material into pellets or fragments and 115 abruptly subjecting the fragments to a coking temperature.

2. The process of making low density carburizing material, which consists in manipulating fine material with a coking binder 120 to produce pellets or fragments and then coking rapidly by initially subjecting the pellets or fragments to a coking temperature.

3. The process of making low density 125 products, which consists in manipulating fine material with a tarry binder to produce pellets or fragments and then coking rapidly.

4. The process of making low density 130

products, which consists in fashioning fine, coking coal, or a mixture containing fine coking coal, into pellets or fragments and then coking rapidly, by initially subjecting 5 the pellets or fragments to a coking temperature.

stantially abrupt application of a coking heat.

20

7. The process of making low density products which consists in fashioning coking material or a mixture containing coking material into pellets or fragments, and rapidly coking the same by initially subjecting 25 them to a tumbling or agitated mass of hot previously coked pellets or fragments maintained at a coking temperature.

In testimony whereof I have hereunto subscribed my name this 2nd day of February, 30 1917.

HUGH RODMAN.

Witnesses:

C. W. McGHEE,  
E. W. McCALLISTER.